

## UNITED STATES PATENT OFFICE

2,057,141

PRODUCTION OF FILAMENTS, THREADS,  
BANDS, RIBBONS AND THE LIKE, FROM  
CELLULOSE DERIVATIVESArthur Eichengrün, Charlottenburg, Germany,  
assignor to Celanese Corporation of America,  
a corporation of DelawareNo Drawing. Application February 5, 1929,  
Serial No. 337,737. In Great Britain February  
8, 1928

2 Claims. (Cl. 18—54)

This invention relates to improvements in the production of filaments, threads, bands, ribbons and the like particularly from cellulose derivatives such as esters or ethers, by extruding suitable solutions of such cellulose derivatives.

For the sake of simplicity the invention will be first described with reference to the production of artificial silk filaments.

The quality of artificial silk filaments produced is at the present time tested by their fineness (denier) and their strength. In order to produce from a given cellulose derivative, for example a cellulose acetate, the desired fineness, i. e., the desired denier, various measures are resorted to, such as for example variation of the size of the spinning aperture, for example, from 0.09 mm. to 0.05 mm., variation of the pressure with which the solution is extruded through the spinning aperture or variation of the temperature of the solution or of the spinning cabinet or finally alteration of the amount of the cellulose derivative in the solution.

It has also been attempted to attain fine filaments by using various different solvents for the cellulose derivatives. Thus for example in my copending application Serial No. 68,707 I have suggested producing artificial silk filaments, threads, bands, ribbons and the like, from a non-inflammable, homogeneous solution having a base of acetone soluble cellulose acetate which has been prepared in the cold by treating said acetate with methylene chloride to which an alcohol or a solvent or a mixture of solvents and a non-solvent for said cellulose acetate or a mixture of two non-solvents which together form a solvent for said cellulose acetate have been added at any suitable stage of said treatment, in amounts compatible with maintaining the mixture non-inflammable.

I have now found a surprisingly simple method of altering the denier of the filaments produced as aforesaid, whilst using the normal spinning apertures, which method may be employed in substitution of or in addition to other known methods of denier regulation such as above-described.

The method of the present invention consists in employing as vehicle for the cellulose derivative, a mixture comprising a lower boiling point solvent or latent solvent (such as acetone or a liquid such as methylene chloride which per se is a non-solvent for said cellulose derivative but nevertheless acts as a solvent therefor in the presence of another liquid) in conjunction with one or more higher boiling point coagulants for

said cellulose derivative, (such as alcohol, benzol or water) and regulating the dimensions of the extruded filaments or the like without altering the size of the extrusion apertures by adjusting the relative amounts of the constituents of the vehicle keeping said cellulose derivative in solution whilst using winding speeds above the normal (namely about 75 metres per minute) and co-relating said winding speeds with the dimensions of the extruded filaments or the like.

Thus for example, in the case of solutions of cellulose acetate in a vehicle comprising methylene chloride as latent solvent such as described in my co-pending application Serial No. 68,707 above referred to, the invention may be carried out by controlling the ratio which the amounts of alcohol constituting the higher boiling coagulant bear to the amount of methylene chloride in said vehicle.

In order to facilitate comprehension of the invention the same will hereinafter be more fully explained with reference to the following examples.

In Example 1 of my co-pending application Serial No. 68,707 I have described the production of artificial silk filaments by the extrusion of a solution of an acetone-soluble cellulose acetate in methylene chloride containing alcohol in amounts compatible with maintaining the mixture non-inflammable. Said application was directed towards the production of a non-inflammable homogeneous solution of cellulose acetate and no particular attention was paid to the amount or proportion of other liquids added to the methylene chloride provided that the solution remained non-inflammable. However, by adjusting, in accordance with the present invention, the amount of the ingredients which together with methylene chloride form the solvent proper for cellulose acetate, it is now possible to reduce the denier of the extruded filament below normal whilst employing the normal spinning apertures.

The results of certain experiments have been set forth in the following tables.

For the sake of comparison I prepared two solutions containing 15 and 20% by weight of cellulose acetate respectively in acetone and solutions containing 15 and 20% by weight of cellulose acetate respectively in mixtures of methylene chloride with alcohol in various proportions. These solutions were extruded through spinning apertures of 0.08 mm. diameter whilst keeping the temperatures, pressures and spinning speeds as uniform

as possible. The denier in each case was measured.

## I

| 5  | Acetone                                  | 15% by weight | 20% by weight |
|----|------------------------------------------|---------------|---------------|
| 10 | Pressure in atmospheres.....             | 32            | 35            |
|    | Temperature °C.....                      | 50            | 45            |
|    | Winding speeds in metres per minute..... | 50            | 64.2          |
| 10 | Denier.....                              | 7.4           | 5.2           |

## II

| 15 | Solvent mixture:<br>85 parts by weight methylene chloride.<br>15 parts by weight alcohol. | 15% by weight | 20% by weight |
|----|-------------------------------------------------------------------------------------------|---------------|---------------|
| 20 | Pressure in atmospheres.....                                                              | 32            | 66            |
|    | Temperature °C.....                                                                       | 50            | 45            |
|    | Winding speeds in metres per minute.....                                                  | 50            | 64            |
| 20 | Denier.....                                                                               | 7.5           | 6.0           |

## III

| 25 | Solvent mixture:<br>75 parts by weight methylene chloride.<br>25 parts by weight alcohol. | 15% by weight | 20% by weight |
|----|-------------------------------------------------------------------------------------------|---------------|---------------|
| 30 | Pressure in atmospheres.....                                                              | 36            | 71            |
|    | Temperature °C.....                                                                       | 48-54         | 40            |
|    | Winding speeds in metres per minute.....                                                  | 95            | 73            |
| 30 | Denier.....                                                                               | 2.6-2.8       | 3.8           |

## IV

| 35 | Solvent mixture:<br>70 parts by weight methylene chloride.<br>30 parts by weight alcohol. | 15% by weight | 20% by weight |
|----|-------------------------------------------------------------------------------------------|---------------|---------------|
| 40 | Pressure in atmospheres.....                                                              | 30            | 70            |
|    | Temperature °C.....                                                                       | 39-41         | 40            |
|    | Winding speeds in metres per minute.....                                                  | 113           | 113           |
| 40 | Denier.....                                                                               | 1.6-1.9       | 3.3           |

## V

| 45 | Solvent mixture:<br>65 parts by weight methylene chloride.<br>35 parts by weight alcohol. | 15% by weight | 20% by weight |
|----|-------------------------------------------------------------------------------------------|---------------|---------------|
| 50 | Pressure in atmospheres.....                                                              | 25            | 80            |
|    | Temperature °C.....                                                                       | 45            | 45            |
|    | Winding speeds in metres per minute.....                                                  | 160           | 156           |
| 50 | Denier.....                                                                               | 1.2           | 2.9           |

From the foregoing tables it will be seen that ordinary solutions of 15 or 20% by weight of acetone-soluble cellulose acetate in acetone respectively give a denier of 7.4 to 5.2, whilst solutions of 15 or 20% by weight of acetone-soluble cellulose acetate in a mixture of 85 parts of methylene chloride and 15 parts of alcohol, give deniers which are respectively not materially altered, viz. 7.5 and 6 respectively. They also show that when the ratio of alcohol to methylene chloride in the solvent mixture is increased the denier is considerably decreased i. e., a much finer thread is obtained, and that the smallest denier or finest thread is obtained when the proportion of alcohol in the solvent mixture is increased to 35%.

The foregoing tables thus demonstrate that the adjustment of the relative proportions of the components forming the vehicle for the cellulose acetate i. e. by increasing the ratio of alcohol (coagulant) to methylene chloride (latent solvent), enables the denier of the extruded filament to be controlled, i. e. reduced and permits of the employment of higher winding speeds.

The filaments produced according to the present invention possess a high "Reisslänge" or 75 "tearing length", (viz. length of freely suspended

filament at which breakage takes place under the influence of the weight of the suspended filament alone).

I have hereinbefore described only the use of 5 solutions containing methylene chloride and alcohol, but it is obvious that the invention may also be carried out with solutions of acetone-soluble cellulose acetate in other solvent mixtures containing for example alcohol, benzol and acetone such as those described in my British specifications Nos. 1441/1910 and 18076/1910, and that by adjusting the relative proportions of the components (e. g. alcohol, benzol and acetone) forming the vehicle of such cellulose acetate the denier 10 of the extruded filament can be modified at will. 15

Similar results can also be obtained with other known solvents and mixtures of solvents and non-solvents or coagulants for cellulose acetate. Thus for example I may employ solvent mixtures consisting of ethylene chloride and alcohol; ethylene 20 chloride, alcohol and acetone; ethyl acetic acetate and alcohol, ethyl formate and alcohol, and may vary the denier by altering the proportion of alcohol. In fact I may even employ a mixture of acetone and alcohol and vary the ratio of alcohol 25 in the mixture in order to modify the denier.

I have also found that instead of modifying the fineness of the thread by modifying the amount of alcohol I can also influence the fineness of the thread by adding small amounts of water with 30 alcohol or other coagulants.

I have above described the application of my invention, to cellulose acetate, however the invention is also applicable to other cellulose derivatives such as other cellulose esters and ethers and 35 cellulose derivatives having inorganic and organic acid radicles, or mixtures of different aliphatic or aromatic acid radicles. For example, I may use ethylcellulose, benzylcellulose and the like, or cellulose-propionate or even mixtures of esters 40 and ethers of aliphatic and aromatic acids. Similar results can also be obtained with alkyl cellulose acetates or nitro-cellulose acetates or mixtures of any of the aforesaid acetates.

The present invention enables perfect filaments 45 of unvarying cross-section to be obtained, presumably by virtue of the fact that when employing a vehicle comprising a rapidly evaporating solvent and a less rapidly evaporating non-solvent or coagulant, the solidifying effect of the 50 atmosphere is rapidly assisted by the effect of the non-solvent after the evaporation of the solvent.

The filaments produced by means of the process of the present invention have been found to have a substantially round shape and to be substantially free from cross-sections of bone shape, such as are usually produced when spinning solutions of cellulose derivatives in a single solvent. 55 Such filaments consequently dye far more evenly and fabric produced therefrom is free from ob- 60 jectionable scintillating effects.

By virtue of the present invention when spinning artificial filaments by a stretch-spinning process, very low deniers can be obtained which are comparable to those obtained in the cupram- 65 monium process.

Whilst I have hereinbefore described the application of the invention only to the production or filaments, it is obvious that the invention can also be applied to the production of threads, 70 bands, ribbons and the like from cellulose derivatives, and the term "filaments" used in the claims includes such threads, bands, ribbons and the like. The breaking length of a filament furnishes a reliable indication of the nature of the 75

bands, ribbons or the like which could be produced by the extrusion of the same solution of cellulose derivative so that it is possible, by varying the ratio of the components of the vehicle, to  
5 vary also the properties of the bands, ribbons or the like produced from such solutions of cellulose derivatives.

It is obvious that innumerable variations and modifications may be made without departing  
10 from the spirit or scope of the invention as defined in the appended claims.

I claim:—

1. Process of producing fine filaments which comprises dissolving cellulose acetate in a mixture  
15 of liquids which is a solvent for the cellulose ace-

tate and which consists substantially of methylene chloride and alcohol, extruding the solution through normal apertures into an evaporative atmosphere, the denier of the filaments being regulated by correlating the winding speeds with 5 the concentration of the solvent and non-solvent constituents in the spinning solution.

2. Process of producing filaments of fine denier which comprises extruding a solution of cellulose acetate in a liquid solvent mixture which consists 10 substantially of methylene chloride and alcohol through normal spinning apertures into an evaporative atmosphere, employing winding speeds of 75 to 160 meters per minute.

ARTHUR EICHENGRÜN. 15